

## UNITED STATES PATENT OFFICE

2,428,603

## PROCESS FOR HARDENING PROTEIN FIBRE

Francis Clarke Atwood, Newton, Mass., assignor,  
by mesne assignments, to National Dairy Products Corporation, New York, N. Y., a corporation of Delaware

No Drawing. Application October 29, 1941,  
Serial No. 417,024

15 Claims. (Cl. 8—127.6)

1

This invention relates to improvements in a process for manufacturing fibres synthetically formed from a proteinaceous material. More particularly, it relates to improvements in that part of the complete process in which the fibre is hardened with formaldehyde subsequent to its spinning and coagulation in an acidic coagulating bath.

The process is applicable primarily to a fibre prepared from casein, such as animal casein obtained from milk, or vegetable casein such as obtained from soybean. However any other alkali-dispersible acid-coagulable protein may be used, such as the alkali-dispersible acid-coagulable proteins derived from cotton seeds, castor beans, natural wool, etc. All of such proteins are dispersible in water with an alkaline material and can be formed into fibre by spinning the dispersion into an acidic coagulating bath. All of these proteins also are hardened by formaldehyde and are therefore adapted for treatment in accordance with this invention.

The complete process, in which my invention is an improvement, includes the step of dispersing the protein with an alkaline material, preferably caustic, but also including other inorganic alkaline materials, such as bases and alkaline salts, ammonia, organic bases, such as the various amines, soaps and similar alkaline materials. This dispersion is accomplished preferably by heating the protein and the alkaline material in a suitable quantity of water to obtain a dispersion of high viscosity. After suitable filtering, centrifuging, cooling and deaerating steps, the dispersion is forced through a spinnerette into an acidic coagulating bath. The composition of this bath preferably includes such a portion of acid as to achieve a relatively low pH value preferably generally within the range of .75 to 2.5 and preferably about a value of 1.50. This bath may also contain a mineral and a vegetable tanning agent such as an alum and "Goulac," respectively, and a soluble salt, such as sodium chloride or sulfate, or both, for dehydration. The fibre is permitted to remain in contact with the acidic coagulating bath for a suitable period and then withdrawn from the bath after which it is permitted to remain wet with the coagulating liquid for a suitable length of time to insure thorough coagulation. Suitable stretching or elongation may be accomplished throughout any portion of this coagulating period.

Following this operation, it has been the practice to treat the fibre to dehydrating and hardening operations. Such operations are accom-

2

plished in one or more baths containing an alkali metal salt of a strong mineral acid, such as sodium chloride or sodium sulfate, a mineral hardening agent such as alum, and formaldehyde in solution. The composition of such a bath or baths may vary over relatively wide limits. It is possible, for example, to use a plurality of baths in which the first contains a relatively smaller proportion of formaldehyde or none at all, and a higher proportion of salt, with or without an alum. Such a bath acts primarily as a hypertonic solution and causes dehydration or shrinking of the fibre, but some hardening action may occur depending on the inclusion and amount of formaldehyde. A subsequent bath or baths may include a much greater concentration of formaldehyde, for example from 7 to 40%, preferably about 10 to 20%. These baths may include a salt and also may include an alum, if desired. The latter is not so essential at this later stage. The salt is preferred in order to maintain the fibre in a dehydrated condition.

The first bath is referred to as a "pickling" bath, particularly if it does not contain any formaldehyde or contains a small amount such as a concentration of under 5%. The second or subsequent baths which contain higher concentrations of formaldehyde for exerting a pronounced hardening action are referred to as hardening baths.

One reason for using two baths instead of one is occasioned by the fact that water is eliminated from the fibre which dilutes the bath. This is undesirable if the bath is to contain a high percentage of formaldehyde. It is preferable to have the dilution occur in the first bath, and to treat the relatively dehydrated fibre with more concentrated formaldehyde. But a single bath may be used if the above disadvantage is of no commercial significance.

In all of these prior proposals, utilizing one or more baths varying in composition as above described and for the purposes above mentioned, there has been no attempt, insofar as I am aware, to control the pH value of the baths within a range which exerts a maximum hardening action. Particularly is this so in the case of the bath or baths containing a relatively large concentration of formaldehyde in which the primary hardening action occurs.

It will be appreciated that the fibre being introduced into these baths is in a very acidic condition because it is wet with the coagulating liquid, and even though an attempt is made to remove the acid which adheres to the surface of the fibre, the fibre is permeated with this acid and at a pH

approximately that of the coagulating liquid. Since relatively large quantities of fibre are passed continuously through these baths, the baths take on the pH value of the fibre or at least are not of such a composition as to alter appreciably the pH value of the fibre. Experience has shown that under actual manufacturing conditions the pH value of the formaldehyde hardening bath will vary from 2.45 to 3.17, depending upon the composition of the bath, the amount of fibre that has been treated in the bath, etc. As far as I am aware, no attempt has been made heretofore to alter the composition of these baths except by varying the salt, alum and formaldehyde content. Such variations do not result in pH values outside of the range mentioned above. While such baths may have a pH value somewhat higher when initially fresh and before any fibre is introduced into them, they very quickly fall to a pH value within the above range as soon as the acid fibre is introduced into them.

I have discovered that a decidedly superior hardening action is obtained if the pH value of the formaldehyde containing bath, such as the pickling and hardening baths, particularly the latter, is controlled and maintained at a pH value of 4.5 or above. The upper limit is not critical but probably should not exceed 7. Very desirable results have been obtained at a pH value of 4.5 and as high as 6.88.

The maintenance of the desired pH value in the so-called pickling bath is more readily achieved, despite the fact that the acidic fibre is introduced into this bath first. The fact that this bath does not contain formaldehyde or an appreciable quantity of it renders it more easily controlled as to pH value. A bath which contains sufficient formaldehyde to exert an appreciable hardening action is much more difficult to control as to pH value and has a more pronounced tendency to remain in an acid condition despite attempts to raise the pH value. This phenomenon may possibly be explained by the action of the formaldehyde on the protein. If it is assumed, as some authorities say, that the formaldehyde acts primarily to block or react with the amino or alkaline groups in the casein or render them inactive, this would render the casein itself more acidic which would tend to maintain the bath in this condition.

The maintenance of this pH value may be accomplished in a number of ways. For example, it is possible to add alkaline material directly to the baths, but this has the danger that portions of the solution will have a pH value higher than the remainder of the bath with consequent non-uniformity of the fibre. It may also be possible to circulate continuously the liquid of the baths through a treating chamber to which appropriate amounts of caustic or carbonates may be added so as to keep the pH value at the desired point. In a continuous operation in which the bath is continuously full of fibre passing therethrough, it is not particularly convenient to use this method. This also has the difficulty that such a control is very difficult since it requires constant analysis, and within this pH range small amounts of caustic may effect an appreciable increase in pH value.

While any method may be used for maintaining the pH value within the range above set forth, and preferably at one point within this range in order that the fibre being processed may be uniform, I prefer to achieve this pH control by means of a buffering salt in the treating baths, particularly the bath containing formaldehyde in a hard-

ening concentration. The buffering salt to be selected will depend somewhat upon the pH value selected.

An alkaline material, such as caustic or soda ash, may be used to raise the pH value to the desired amount, in combination with an appropriate buffering salt to hold the solution at about the pH value achieved by the addition of the alkaline material.

An alkali metal acetate, such as sodium acetate, is very desirable when the pH range is to be maintained in the neighborhood of 4.5 to about 5.5 or possibly 6.0 under certain circumstances.

In an embodiment of my process that is particularly practical under present day manufacturing conditions, the pickling solution may comprise an aqueous solution containing 3 to 15%, preferably 5 to 10% of a soluble salt, such as sodium sulfate or sodium chloride, or both, formaldehyde in an amount 0 to 5%, preferably 1 to 3%, and sodium acetate and alkaline materials in amounts to achieve and maintain a pH value within the range of 4.5 to 5.2. The hardening bath may contain formaldehyde in an amount of 5 to 40%. Concentrations as high as the upper limit are not required, however, for good results, and a range within 7 to 10% is desirable for satisfactory results. To this solution is added sodium acetate and alkaline materials in such amounts as to achieve and maintain a pH value within the range of 4.5 to 5.2. If desired other soluble salts, such as sodium chloride or sodium sulfate or both, may be included, but this is not so essential for a hardening solution, although desirable to maintain the fibre in a dehydrated condition. Alum may also be added but is generally not necessary.

When utilizing a higher pH value, this is obtained by the use of other buffering salts, as is well known in the art; for example, suitable proportions of citric acid and di-sodium phosphate, and also suitable proportions of mono-sodium di-acid phosphate and di-sodium mono-acid phosphate. The mere addition of tri-sodium phosphate to an acid solution may accomplish this.

While I have selected the range of 4.5 to 5.2 as a commercial operating range, this is done primarily because a pH within this range gives satisfactory results and is readily obtained as a practical matter by using sodium acetate as a buffering salt. Ranges as high as 7 give equally good, and probably superior results, as indicated hereinafter, particularly if a rapid reaction is desired.

As indicative of the results that may be obtained in accordance with my invention, a fibre prepared in the conventional manner by hardening it in an ordinary bath containing 20% formaldehyde, 5% salt and 5% alum and having a pH value of 1.5, was compared with a fibre hardened in a bath containing 20% formaldehyde and other ingredients similar but having the pH value of 6.5. The samples of fibre treated in the two baths showed a remarkable difference in the permanency of the fibre formation. After one hour of treatment in the ordinary bath, the fibre is harsh and welded together, whereas in the hardening bath having the pH value of 6.5, the fibre is soft, open and readily carded upon drying. It is also observed that the fibre from the ordinary hardening bath is easily stretched and rubbery, whereas the fibre formed in the bath with a higher pH value is more firm and of a fibrous nature.

These results were checked by comparing the fibre treated in baths such as mentioned above

but having pH values of 2.7 and 5.7, respectively. The results were quite similar.

As further illustrative, the following example is given with reference to a bath containing a lower concentration of the formaldehyde. A bath containing 7% formaldehyde, 2½% salt, 2½% alum, and having a pH value of 3.45 was compared with a similar hardening bath containing the same amount of formaldehyde but buffered to a pH value of 6.56. A comparison of the fibres treated in these two baths shows that in the more acidic bath after one hour treatment, the fibre was brittle and welded together, whereas after hardening in the bath of higher pH value for twenty minutes, a fibre was obtained which was soft, not welded, and readily carded. This indicates that much lower concentrations of formaldehyde may be used upon increasing the pH value of the formaldehyde bath. In a commercial operation operating at a pH value of 6.0, a formaldehyde concentration of 5% gives excellent results.

As a further example, a hardening bath containing 18% formaldehyde and without any salt or alum was adjusted to a pH value of 3.5; a fibre treated therein for one hour and dried resulted in a brittle welded mass; a fibre treated in an identical bath but buffered to a pH value of 6 was an excellent fibre in every respect. This indicates that upon proper control of the pH value, the amount of salt or alum in the hardening bath may be greatly reduced if not entirely eliminated, and the time of reaction may be greatly shortened.

I have also discovered that when utilizing formaldehyde baths in which the pH value is controlled as above noted, that superior results are obtained if the temperature is maintained within relatively critical limits; and also a much more shorter treating operation is required. While the desirable results in accordance with my invention may be obtained utilizing a bath at room temperature, providing the treatment is prolonged somewhat, I have ascertained that the maximum speed in hardening and the greatest superiority in the fibre is obtained if a temperature range of from 100 to 125° F., preferably 115 to 120° F. is maintained in the formaldehyde hardening bath. Investigations indicate that a bath containing 5% formaldehyde buffered to a pH value of 6.0 or 6.5 and at a temperature of 115 to 120° F. gives a satisfactory hardened fibre in 10 to 30 minutes. This is to be compared with the prior art known requirements of from 10 to 12 hours.

I have also discovered that when utilizing a formaldehyde bath maintained at the above pH value and preferably within preferable temperature ranges, that desirable results are obtained with respect to strength and fibre diameter if the fibre is kept at constant length while in the bath or baths so that it is not permitted to shrink, particularly in the case of the hardening bath. This action is referred to more generally as tensioning. While the fibre may actually be elongated during this treatment, it is practical that the fibre, while in the hardening bath, may be suspended between rollers or run in loops between rollers or other suitable means whereby it is maintained at the same length during the treatment in the bath and thus preventing shrinkage. As further illustrative of this aspect of my invention, a fibre which is introduced into an ordinary hardening bath at the rate of 220 feet per minute and permitted to stand in the bath for one hour without being subjected to

any tension, would be withdrawn from the bath at the rate of 150 to 170 feet per minute. This indicates the shrinkage in length of the fibre that takes place during the hardening. If the fibre, while it is in the hardening bath, is maintained at constant length, such as passing it continuously between rollers so as to be in loops of fixed lengths, whereby the continuous strand entering and leaving the hardening bath moves at the same rate, it has been found that the fibre is greatly improved in strength and is of a much smaller desirable diameter. The results are indicated in the following table:

| 15 | Sample No. | Tension During Hardening | Strength in Pounds per Square Inch | Diameter in Microns |
|----|------------|--------------------------|------------------------------------|---------------------|
| 1  |            | No.                      | 10,890                             | 16.8                |
| 1  |            | Yes.                     | 12,600                             | 12.4                |
| 2  |            | No.                      | 10,740                             | 20.2                |
| 2  |            | Yes.                     | 16,084                             | 15.9                |
| 3  |            | No.                      | 11,950                             | 19.4                |
| 3  |            | Yes                      | 14,130                             | 15.7                |

From the above it will be seen that an increase in strength from 15 to 50% is obtained and a reduction in fibre diameter of about 25%.

Throughout this specification I have indicated what I believe to be the upper and lower critical limits of the various factors when such limits are critical for securing the new results in accordance with my invention. I have also included a more limited range which I regard as the optimum conditions either from the commercial standpoint or for securing the most favorable results. The inclusion of a statement of the optimum conditions in order that my invention may be practiced with the greatest benefit and advantage is not intended to be inconsistent with the critical nature of the range over which the new result may be obtained.

Fiber made in accordance with the invention is admirably suited for treatment in subsequent processes such as acylating with ketene or acetic anhydride, deaminizing by nitrous acid, etc.

It will be obvious that many variations may be made within my invention as outlined above and that various expedients apparent to those skilled in the art may be resorted to for carrying into effect the invention as described herein.

I intend all such equivalents and variations to be included within the scope of my invention.

This application is a continuation-in-part of application Serial No. 309,028, filed December 13, 1939, now Patent No. 2,342,994.

55 I claim:

1. In a process of hardening a proteinaceous fibre that has been formed from an alkali-dispersible acid-coagulable protein by dispersing said protein with an alkaline material and spinning the dispersion into an acidic coagulating bath whereby the fibre is impregnated with the acid in said bath, following which the fibre is stretched; the steps which comprise placing said acid coagulated and stretched fibre in a hardening bath containing formaldehyde, and maintaining the pH value of said bath at not less than 4.5 and not more than 7.0 during which time the fibre is hardened in said bath.

2. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the step which comprises hardening said coagulated and

stretched fibre in a formaldehyde hardening bath maintained at a temperature of 100 to 125° F., and at a pH value of not less than 4.5 and not over 7.0.

3. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the step which comprises hardening said coagulated and stretched fibre while maintained against shrinkage in a formaldehyde hardening bath having a temperature of 100 to 125° F. and a pH value of not less than 4.5 and not over 7.0.

4. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the step which comprises hardening said coagulated and stretched fibre in a hardening bath containing formaldehyde in a concentration of at least 5% and buffered at a pH value of not less than 4.5 and not over 7.0 by a buffering salt.

5. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the step which comprises hardening said coagulated and stretched fibre in a hardening bath containing formaldehyde in a concentration of at least 5% and maintained at a pH value of not less than 4.5 and not over 7.0 by the buffering action of sodium acetate included in said bath.

6. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the step which comprises hardening said coagulated and stretched fibre in a hardening bath containing formaldehyde in a concentration of at least 5% and maintained at a temperature of 100 to 125° F., and a pH value of not less than 4.5 and not over 7.0 by a buffering salt.

7. In a process of hardening a casein fibre that has been formed by dispersing said casein with an alkaline material, spinning the dispersion into an acidic coagulating bath, and stretching the coagulated fibre; the step which comprises hardening said fibre while maintained against shrinkage in a hardening bath containing formaldehyde in a concentration of at least 5% and maintained at a temperature of 100 to 125° F., and a pH value of not less than 4.5 and not over 7.0 by the buffering action of sodium acetate included in said bath.

8. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the steps which comprise introducing said coagulated and stretched fibre into a first stage hardening bath containing not more than 5% formaldehyde, and 3 to 15% of an alkali metal salt of a strong mineral acid, and having a pH value of not less than 4.5 and not over 7.0; and transferring the preliminarily hardened fibre to a second stage hardening bath containing at least 5% formaldehyde and buffered to a pH value of not less than 4.5 and not over 7.0 by means of sodium acetate.

and buffered to a pH value of not less than 4.5 and not over 7.0.

9. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the steps which comprise introducing said coagulated and stretched fibre into a first stage hardening bath containing not more than 5% formaldehyde, and 3 to 15% of an alkali metal salt of a strong mineral acid and buffered to a pH value of not less than 4.5 and not over 7.0 by a buffering salt, and transferring the preliminarily hardened fibre to a second stage hardening bath containing at least 5% formaldehyde and buffered to a pH value of not less than 4.5 and not over 7.0 by a buffering salt.

10. In a process of hardening a proteinaceous fibre that has been formed from an alkali-dispersible acid-coagulable protein by dispersing said protein with an alkaline material, spinning the dispersion into an acidic coagulating bath, and stretching the coagulated fibre; the steps which comprise introducing said coagulated and stretched fibre into a first stage hardening bath containing not more than 5% formaldehyde, and 3 to 15% of an alkali metal salt of a strong mineral acid, and having a pH value of not less than 4.5 and not over 7.0, and transferring the preliminarily hardened fibre to a second stage hardening bath containing at least 5% formaldehyde and maintained at a temperature of 100 to 125° F. and a pH value of not less than 4.5 and not over 7.0.

11. In a process of hardening a casein fibre that has been formed by dispersing said casein with an alkaline material, spinning the dispersion into an acidic coagulating bath, and stretching the coagulated fibre; the steps which comprise introducing said coagulated and stretched fibre into a first stage hardening bath containing not more than 5% formaldehyde, and 3 to 15% of an alkali metal salt of a strong mineral acid, and having a pH value of not less than 4.5 and not over 7.0, and transferring the preliminarily hardened fibre to second stage hardening bath containing at least 5% formaldehyde and buffered to a pH value of not less than 4.5 and not over 7.0 by means of sodium acetate.

12. In a process of hardening a casein fibre that has been formed by dispersing said casein with an alkaline material, spinning the dispersion into an acidic coagulating bath, and stretching the coagulated fibre; the steps which comprise introducing said coagulated and stretched fibre into a first stage hardening bath containing not more than 5% formaldehyde, 3 to 15% of sodium chloride, and buffered to a pH value of not less than 4.5 and not over 7.0 by sodium acetate, and transferring the preliminarily hardened fibre to a second stage hardening bath containing at least 5% formaldehyde and maintained at a temperature of 100 to 125° F. and buffered to a pH value of not less than 4.5 and not over 7.0 by means of sodium acetate.

13. In a process of hardening a casein fibre that has been formed by dispersing said casein with an alkaline material and continuously spinning the dispersion into an acidic coagulating bath whereby the fibre is impregnated with the acid in said bath, following which the coagulated fibre is stretched; the steps which comprise continuously introducing said acid coagulated and

stretched fibre into a first stage hardening bath containing not more than 5% formaldehyde, 3 to 15% sodium chloride and buffered to a pH value of 4.5 to 5.2 by the inclusion of sodium acetate in said pickling bath and the neutralization of any acid introduced with the fibre into said bath, permitting the fibre to remain in said bath for from 10 to 60 minutes, continuously removing the fibre from said bath and transferring the preliminarily hardened fibre to a second stage hardening bath containing at least 5% formaldehyde, 5 to 15% sodium chloride, and maintained at a temperature of 110 to 125° F. and buffered to a pH value of 4.5 to 5.2 by means of sodium acetate.

14. In a process of hardening a proteinaceous fibre that has been formed from an alkali-dispersible acid-coagulable protein by dispersing said protein with an alkaline material and spinning the dispersion into an acidic coagulating bath whereby the fibre is impregnated with the acid in said bath, following which the coagulated fibre is stretched; the steps which comprise continuously introducing said acid coagulated and stretched fibre into a hardening bath containing formaldehyde and an alkali metal salt of a strong acid, and maintaining the pH value of said last-mentioned bath at not less than 4.5 and not over 7.0 by neutralizing any acid introduced into said bath by said fibre and by incorporating in said bath an alkali metal salt of a weak acid.

15. In a process of hardening a proteinaceous fibre that has been formed from an alkali-dispersible acid-coagulable protein by dispersing said protein with an alkaline material and spinning the dispersion into an acidic coagulating bath whereby the fibre is impregnated with the acid in said bath, following which the coagulated fibre is stretched; the steps which comprise continuously introducing said acid coagulated and stretched fibre into a first stage hardening bath containing a small amount of formaldehyde and alkali metal salt of a strong mineral acid, main-

taining the pH value of said bath at not less than 4.5 and not over 7.0 by incorporating therein buffering salt and by neutralizing any acid introduced into said bath by said acid coagulated fibre; continuously transferring the fibre to a second stage hardening bath containing at least 5% formaldehyde and an alkali metal salt of a weak acid to maintain said bath buffered to a pH value of not less than 4.5 and not over 7.0.

FRANCIS CLARKE ATWOOD.

#### REFERENCES CITED

The following references are of record in the file of this patent:

#### UNITED STATES PATENTS

| Number       | Name     | Date          |
|--------------|----------|---------------|
| 2,266,672    | Wormell  | Dec. 16, 1941 |
| 2,167,570    | Heckel   | July 25, 1939 |
| 2,211,961    | Meigs    | Aug. 20, 1940 |
| 2,290,789    | Wormell  | July 21, 1942 |
| 2,312,998    | De Kadet | Mar. 2, 1943  |
| 2,338,916    | Ferretti | Jan. 11, 1944 |
| 25 2,338,917 | Ferretti | Jan. 11, 1944 |

#### FOREIGN PATENTS

| Number     | Country       | Date          |
|------------|---------------|---------------|
| 30 510,131 | Great Britain | July 27, 1939 |
| 502,710    | Great Britain | Mar. 23, 1939 |

#### OTHER REFERENCES

Brother and McKinney, Protein Plastics From Soybean Products from "Ind. and Eng. Chem.," 35 Nov. 1938, pgs. 1236-40.

La processus de durcissement dans l'industrie de la galalithe J. Delorme—Rev. Gen. Mat. Plastiques, 1936, T. 12, No. 3, pgs. 74-76, Mars. from Chemie and Industrie, Cas. Dig.

Mougeot, Formaldehyde in the Hardening of Casein Objects from "Rev. Gen. des Matieres Plastiques," Feb. 1928, vol. 14, No. 2, pages 35-37.

**Certificate of Correction**

Patent No. 2,428,603.

October 7, 1947.

**FRANCIS CLARKE ATWOOD**

It is hereby certified that errors appear in the printed specification of the above numbered patent requiring correction as follows: Column 7, line 56, claim 7, after the word "said" insert *coagulated and stretched*; column 8, line 48, claim 11, for "to second" read *to a second*; column 9, line 25, claim 14, for "alklai" read *alkali*; column 9, line 15, beginning with "In a process" strike out all to and including the word and period "acid." in line 30, comprising claim 14, and insert the same after claim 1, as claim 2; same column, line 31, beginning with "In a process" strike out all to and including the numeral and period "7.0" in column 10, line 9, comprising claim 15, and insert the same after claim 8, as claim 10; and for the claim numbers "2", "3", "4", "5", "6", "7", "8", "9", "10", "11", "12", and "13", read *3, 4, 5, 6, 7, 8, 9, 11, 12, 13, 14, and 15*, respectively; and that the said Letters Patent should be read with these corrections therein that the same may conform to the record of the case in the Patent Office.

Signed and sealed this 27th day of January, A. D. 1948.

**[SEAL]**

**THOMAS F. MURPHY,**  
*Assistant Commissioner of Patents.*